

Patented Nov. 4, 1930

1,780,594

150

## UNITED STATES PATENT OFFICE

RALPH E. LAWRENCE, OF WICKLIFFE, OHIO, ASSIGNOR TO THE GRASSELLI CHEMICAL COMPANY, OF CLEVELAND, OHIO, A CORPORATION OF DELAWARE

## ACID TREATMENT OF METAL ARTICLES

No Drawing.

Application filed October 9, 1929. Serial No. 398,505.

This invention relates to inhibitors used in acid treatments of metal articles to prevent, or at least minimize, the action of the acid upon the metal itself, without impairing the action of the acid upon oxides, rust, scale, salts or other undesirable incrustation and corrosion products deposited on the surface of the articles.

I found that thioglycollic acid and certain of its derivatives have to a marked degree an inhibiting effect upon the action of acids upon metals.

Thioglycollic acid, which is easily prepared from chloracetic acid and sodium hydrogen sulfid has the formula:



It forms easily thio-esters, for instance, ethyl-thioglycollic acid:



the action of chloracetic acid upon sodium sulfid forms di-thio-glycollic acid:



and this latter, in common with most organic compounds having an S atom between two C atoms, forms polysulfides by addition of sulfur to the S between the carbon atoms; these compounds are characterized by having in common the same radical:



35 and it seems that this radical is, in this class of substances, the determining factor in developing the inhibiting property. As a matter of fact thioglycollic acid, its salts and esters, thio-di-glycollic acid, its salts, etc., poly-thio-glycollic acids and similar substances containing in their molecule the radical



45 display to a varying, and in some instances to a very marked degree, the property of inhibiting the action of acids upon metals.

It is at the present time understood that the action of the inhibitors generally functions mainly in relation to the hydrogen ion

of an acid bath and is practically independent of the anion; this is also believed to be true with the novel inhibitors of my present invention, as I found that the thioglycollic acid and its derivatives display 55 their inhibiting action with various non-oxidizing acids, such as dilute sulfuric, hydrochloric, acetic, etc., acids, solutions of acid sulfates, etc., which are commonly used in acid metal cleaning operations. 60

Various non-oxidizing acids are used in different concentrations and under different conditions in metal pickling and cleaning operations. The application of my invention to these operations does not necessitate 65 any material change in the composition of the acid baths therein, except the addition to such baths of small amounts of my inhibitors. As a rule amounts of  $\frac{1}{2}$  of 1%, or less of a thioglycollic acid or its derivative 70 is sufficient to insure a far going protection of the metal against attack, or corrosion of the metal itself without affecting the dissolution of acid soluble incrustations on the articles. Some of my novel inhibitors are difficult soluble in the dilute acid baths used and it is therefor necessary to provide for a uniform distribution of the inhibitor throughout the bath in a finely-divided form. This is easily achieved by adding it in the 75 form of a water soluble salt or mixing it first with concentrated acid, such as sulfuric. It is also possible to mix the inhibitor first with a protective colloid and foaming agent. When such compounded inhibitors are added 80 to the dilute acid they will precipitate uniformly and in fine suspension and insure their most efficient action.

The efficiency of inhibitors is conveniently 90 determined by laboratory tests involving the measurement under comparative conditions of the gas evolved from a standard piece of steel immersed in dilute sulfuric acid containing various amounts of the inhibitor.

The results tabulated below have been obtained from pieces of black, mild steel sheet of about 8 square inches surface immersed at room temperature in 34% sulfuric acid and give the amount of gas evolved in cc. 95 100

| Amount of inhibitor                           | 0.5% |   | 0.1% |    | 0.05% |      |
|-----------------------------------------------|------|---|------|----|-------|------|
| Hours of immersion                            | 1    | 2 | 6    | 20 | 1     | 2    |
| Thioglycollic acid                            |      |   |      |    | 6     | 20   |
| Ethyl-thio-glycollic acid                     | 3    | 3 | 3    | 7  | 121   | >350 |
| Thio-diglycollic acid                         |      |   |      |    | 20    | 80   |
| Poly-thio-glycollic acid                      |      |   |      |    | 31.50 | >350 |
| Same first dispersed in 60° Be. sulfuric acid |      |   |      |    | 34.60 | 200  |
|                                               |      |   |      |    | 8     | 11   |
|                                               |      |   |      |    | 40    | 57   |

10 The evolution of gas in a blank test containing no inhibitor was already considerably more than 400 cc. after 6 hours immersion.

I claim:

1. In a process of pickling and cleaning metal articles which comprises subjecting said articles to an acid bath containing as the active pickling and cleaning ingredient a non-oxidizing acid, the step of inhibiting the action of said acid upon the metal by the incorporation into said acid of an inhibitor of the class of substances comprising thio-glycollic acid and its derivatives containing the radical  $\text{COOH}-\text{CH}_2-\text{S}$ .

2. In a process of pickling and cleaning metal articles which comprises subjecting said articles to an acid bath containing as the active pickling and cleaning ingredient a non-oxidizing acid, the step of inhibiting the action of said acid upon the metal by the incorporation into said acid of an inhibitor of the class of substances comprising thio-glycollic acid and its derivatives containing the radical  $\text{COOH}-\text{CH}_2-\text{S}$  finely dispersed throughout said bath.

3. A composition of matter for pickling and cleaning metal articles comprising a dilute non-oxidizing acid and a small amount of an inhibitor of the class of substances comprising thio-glycollic acid and its derivatives containing the radical  $\text{COOH}-\text{CH}_2-\text{S}$ .

40 4. A composition of matter for pickling and cleaning metal articles comprising a dilute non-oxidizing acid and a small amount of an inhibitor of the class of substances comprising thio-glycollic acid and its derivatives containing the radical  $\text{COOH}-\text{CH}_2-\text{S}$ , finely dispersed throughout said acid.

In testimony whereof, I affix my signature.  
RALPH E. LAWRENCE.